

## UNITED STATES PATENT OFFICE.

CHARLES CUMINGS, OF CHICAGO, ILLINOIS.

## STEEL.

No Drawing.

Application filed December 10, 1921. Serial No. 521,476.

*To all whom it may concern:*

Be it known that I, CHARLES CUMINGS, a subject of the King of Great Britain, residing at Chicago, in the county of Cook and 5 State of Illinois, have invented certain new and useful Improvements in Steel, of which the following is a specification.

The invention relates to steel and has as an object the provision of a form of steel 10 which has much improved physical properties and capabilities of working as compared with the steel at present known.

The steel provided by the present invention may be produced by the process disclosed in my application Serial Number 347,004, filed December 23, 1919. Briefly stated the process there described comprises the treatment of the steel in its molten condition by subjecting the same to the effects 20 of an explosion followed by a violent agitation, and preferably accompanied by a substantial rise in temperature.

The physical appearance of the improved steel does not differ in any substantial particular from that already known with the possible exception that the fractures when the metal is broken in a testing machine usually have a more perfect cup and cone form, and the crystallin structure upon the end of 30 the fracture is usually more of a silky nature and of finer appearance than the forms of steel heretofore known when not containing alloys of rare metals.

In the cast condition the tensile strength 35 of the improved steel increases with each .10% of carbon by from 8,000 pounds per square inch upwards, as compared with an average increase of 6,000 pounds in carbon steel as heretofore manufactured. By carbon steel I intend to indicate a steel containing only very small percentages, if any, of the metals commonly alloyed with steel to improve its physical properties, such as tungsten, chromium, nickel, etc.

45 As heretofore produced by the best known commercial methods carbon steel in its condition as cast and normalized has had an average tensile strength with .20% carbon of about 52,400 pounds per square inch and 50 with 50% carbon of about 71,000 pounds per square inch. The improved steel of the present invention under like treatment with the exception of the process described in my copending application above referred to, and

with substantially the same chemical analysis shows for .20% C. a tensile strength of approximately 70,000 pounds per square inch and for .50% C. a tensile strength of approximately 100,000 pounds per square inch. Not only has the improved steel a high tensile strength as compared with steel heretofore known but its elastic limit is higher in proportion to its tensile strength being approximately 80% thereof. The elastic limit of carbon steels heretofore known has 60 been about 70% of its tensile strength. The Brinnell hardness of the improved steel is also greater than the steel of the prior art of like chemical composition. Carbon steel as heretofore known increases in tensile 70 strength under heat treatment and forging by 40 to 75%. Like treatment of the improved steel results in an increase of from 50 to 100%.

Photomicrographs of the improved steel show clearly a greatly reduced number of slag inclusions and those that are found in the metal as cast, in substantially every instance, are in the form of spheres showing as circles on the etched samples. Steel heretofore made contained its slag inclusions in various irregular forms elongated in all directions, which forms have a very much more deleterious effect upon the strength of the steel than do inclusions in the form of spheres. The reference in the claims to a substantial freedom from slag is intended to refer to the comparative freedom as compared with steel heretofore known and not to an actual absence of any slag inclusions. 90

It is found that the improved steel yields more readily to heat treatment than steel of like chemical composition heretofore known. That is to say, the time required for the point of decalescence while the temperature of the steel is being raised is much shorter than former steels of like chemical composition. After the steel is normalized it may be raised to a much higher temperature 95 without injury than has been the case with former steels and the resulting wider range of temperatures which may be applied in heat treatment results in a reduced liability of injury.

When the improved steel is poured from the furnace into the ladle or mould it pours much more quietly and is found to flow more readily in casting than steel hereto-

fore known. As the result of this quality very thin sections may be cast without liability to blow-holes or cavities.

It is found that the readiness with which 5 the steel forges is much improved, and that during machining operations it cuts more smoothly, leaving edges which have not the torn appearance which sometimes appears with steel now in use. The improved action 10 on forging and shaping by cutting is believed to be due to the more homogeneous structure and to the finer grain of the steel which qualities are plainly exhibited by photomicrographs of etched samples. In the 15 normalized state the pearlite shown by such samples shows a structure approaching the sorbitic rather than lamellar, as is usual in steels under like conditions. "Normalize" as used herein and in the claims is intended 20 to refer to heating the steel to a temperature above the point of decalescence and slowly cooling.

Minor changes may be made in the steel 25 from the physical properties claimed in the following claims without departing from the spirit of the invention.

I claim:

1. A carbon steel the elastic limit of which is at least 80% of its tensile strength.
2. A carbon steel which after being normalized and subsequently heated to a temperature above its point of decalescence and

quenched has its tensile strength increased at least 100% by the heat treatment.

3. A carbon steel which after being normalized and subsequently heated to a temperature above its point of decalescence and quenched has its tensile strength increased at least 75% by the heat treatment.

4. A carbon steel having not more than .50% carbon, which when cast and normalized, has a tensile strength of at least 90,000 pounds per square inch.

5. A carbon steel having not more than .50% carbon, which when cast and normalized has a tensile strength of at least 100,000 pounds per square inch.

6. A series of carbon steels of varying proportions of carbon, the individuals of said series having a tensile strength which varies by at least 8,000 lbs. per square inch with each difference of .10% of carbon.

7. A carbon steel made by the process herein referred to which in normalized condition has its tensile strength increased at least 8,000 pounds per square inch by an addition of .10% of carbon.

8. A carbon steel made by the process herein referred to which in normalized condition has its tensile strength increased at least 10,000 pounds per square inch by an addition of .10% of carbon.

CHARLES CUMINGS.